

C. A. CADWELL.  
RAIL BOND AND METHOD OF MAKING SAME.  
APPLICATION FILED JUNE 23, 1919.

1,412,269.

Patented Apr. 11, 1922.



INVENTOR  
Charles A. Cadwell  
By Day, Oberlin & Day.  
ATTORNEYS.

# UNITED STATES PATENT OFFICE.

CHARLES A. CADWELL, OF CLEVELAND, OHIO, ASSIGNOR TO THE ELECTRIC RAILWAY IMPROVEMENT COMPANY, OF CLEVELAND, OHIO, A CORPORATION OF OHIO.

## RAIL BOND AND METHOD OF MAKING SAME.

1,412,269.

Specification of Letters Patent. Patented Apr. 11, 1922.

Application filed June 23, 1919. Serial No. 306,172.

To all whom it may concern:

Be it known that I, CHARLES A. CADWELL, a citizen of the United States, and a resident of Cleveland, county of Cuyahoga, and State of Ohio, have invented a new and useful Improvement in Rail Bonds and Methods of Making Same, of which the following is a specification, the principle of the invention being herein explained, and the best mode in which I have contemplated applying that principle, so as to distinguish it from other inventions.

Heretofore, in order to satisfactorily apply a solid terminal or head to a flexible conductor, as in the manufacture of rail bonds and the like, it has been found necessary to separately cast such terminal and then forge or swage the same on the end of the conductor in order to secure a firm union between the same, and at the same time compact the material of the head. The object of the present invention is to provide a method for directly casting such terminals or heads in place on the end of the conductor so as not only to effect a homogeneous juncture between the individual strands of the latter and such head, but also provide a head possessing sufficient density and proper texture to serve without further treatment or manipulation as a finished terminal.

In order to effect a welded union between wires or laminations of a conductor and molten metal added to form a terminal, heat must be applied in quantity sufficient that the ends of the wires be brought to the melting point. The metal, copper, is peculiar in the fact that it has no plastic or pasty condition as it approaches the melting temperature, but disintegrates from the solid state to beads of melted copper which exude from the solid, leaving a porous brittle structure which is commonly called burnt copper, and is generally known to be very weak mechanically. Casting copper directly upon the wires of a copper conductor to form a terminal may give a poor result from lack of sufficient heat to form any kind of a union, and at best the union obtained is subject to the criticism above mentioned. However, by the present method of arc-melting the metal for the terminal directly into a mold, the amount of heat required to form a perfect union of the metals, can be accurately con-

trolled, and by adding to the ends of the copper conductor after it is placed in the 55 mold a small quantity of spelter solder or hard solder, an alloy metal is formed at the point of union which is free from the weakness of the all copper weld.

My improved method may be used for 60 welding the terminal to the conductor and to the rail, thus simultaneously forming the bond and installing it; or to the conductor alone, in order to form a bond designed to be installed on the rail by mechanical means 65 or by soldering, brazing or welding.

To the accomplishment of the foregoing and related ends, the invention, then, consists of the steps and means hereinafter fully described and particularly pointed out in 70 the claims, the annexed drawing and the following description setting forth in detail certain means and one mode of carrying out the invention, such disclosed means and mode illustrating, however, but one of 75 various ways in which the principle of the invention may be used.

In said annexed drawing:—

Fig. 1 is a plan view of a suitable apparatus including a mold and welding pencil 80 for forming terminals directly on the ends of conductors, in accordance with my present improved method; Fig. 2 is a view of an apparatus similar to that of Fig. 1, but showing a modification consisting in the incorporation in the terminal of a plate of 85 steel or other metal within the copper which composes the head or terminal proper; Fig. 3 is a plan view of a modified form of mold for forming a different type of terminal, i. e. 90 a stud terminal on the end of the conductor; Fig. 4 is a central vertical section of such modified form of apparatus, the plane of the section being indicated by the line 4—4, Fig. 3; Fig. 5 is a plan view showing still 95 another form of apparatus adapted for the casting of the terminal and at the same time applying the same to the rail to which it is to be attached; Fig. 6 is a transverse section through such rail and associated apparatus, the plane of the section being indicated by the line 6—6, Fig. 5; Fig. 7 is a longitudinal section through the end of the 100 cable or specially prepared conductor which enters into the operation and forms part of 105 the bond when completed; Fig. 8 is a longi-

tudinal section of a finished bond terminal of the kind formed in the apparatus of Fig. 1; while Fig. 9 is a similar section of a finished terminal of the kind formed by the 5 apparatus of Fig. 2.

The method consists essentially in inserting the end of a flexible copper band into a suitable open chill mold, covering the end so inserted, with a mixture of powdered 10 brazing material and finely cut or granulated copper and then simultaneously fusing together the end of the copper conductor, the brazing material and granular copper and additional copper added by the arc 15 pencil, by means of which the fusing and brazing is done.

The arc pencil may consist of a rod of copper which melts away as the operation proceeds, or it may consist of a carbon 20 pencil, the operator feeding in a rod of copper as the operation progresses. The copper pencil is adapted to be used either for forming and installing the bond on the rail, or for forming a bond designed to be subsequently 25 installed on the rail by other means. The carbon pencil, however, can be used only by giving it a negative polarity, which means that it is not applicable to the direct welding of the conductor to the rail, if the 30 electric current used is taken directly from the trolley through a rheostat.

The conductor usually employed in bonding operations is of stranded form, being shown in the several figures of the drawings 35 as consisting of a section 1 of copper cable. The end 2 of such section designed to enter into the terminal is compressed and preferably more or less flattened to approximate in form the desired cross-section of the head 40 or terminal. Previously to such compression a sleeve 3, likewise of copper, is fitted over the end of the conductor and is flattened down along with the latter. This terminal is then laid in a recess in a block of 45 suitable refractory material, so as to leave a portion of the sleeve lie clear of such mold, the unfilled portion of the recess being of any desired shape or size. Thereupon molten copper is deposited in the recess, and upon the exposed ends of the conductor as well as the adjacent, i. e. outer, end of the sleeve, so as to fuse such strands and sleeve together, forming a homogeneous 50 mass of the same, along with the metal deposited in the recess. Preferably the molten metal is derived from a copper pencil 4 which forms one terminal of an electric circuit 5, the mold constituting the other, so that an arc is formed between such pencil 55 and mold, causing the end of the latter to gradually melt down.

The form of mold 7 illustrated in Fig. 1 is obviously designed to provide a head or terminal of flat form having a cross-section 60 approximately the same as that of the flat-

tened compressed end of the stranded conductor (see Fig. 8). In Fig. 2 the mold 8 is of substantially the same character, the modification consisting in the introduction in such mold, preliminarily to the addition 70 of the copper, of a plate 9 of steel or other ferrous metal, the same being disposed so as to be incorporated in the face of the finished terminal that is designed to be applied to the rail. (See Fig. 9.) This plate 9 is 75 homogeneously united with the finished terminal under the influence of the molten metal deposited in the recess back of it.

In Figs 3 and 4, as already indicated, the modification consists in the form of the 80 mold recess 10 which here includes a cylindrical depression 11 whereby the head or terminal proper is formed with a corresponding projecting stud.

In the apparatus shown in Figs. 5 and 6, 85 the mold 12 is formed with a wall on the one side only of the recess, the other being closed by the side of the rail 13, when such mold is pressed against the latter, thus causing the end 2 of the conductor to be pressed against 90 such adjacent rail face when it is inserted in the recess in the fashion heretofore described. The result of melting down the pencil in this case is to not only form a head or terminal on the end of the conductor as 95 heretofore described, but at the same time to homogeneously unite such head with the adjacent rail face. As a result, when the mold is removed the conductor is left attached to the rail through the medium of 100 the head or terminal thus formed.

A certain amount of braze 14, preferably in granular or dust form, is applied to the ends of the strands of the conductor which project into the recess in each of the forms 105 of apparatus illustrated in Figs 1, 2, 3 and 4. In order that such braze may be conveniently provided in proper amount in the case of the form of apparatus illustrated in Figs. 5 and 6, the end of the sleeve 15 is 110 here prolonged beyond the ends of such strands, and the bronze or braze 16 is deposited inside such sleeve extension 17, after which the walls of the latter are closed together so as to retain the braze material 115 until the molten metal from the pencil is applied.

The sectional views of the completed terminal appearing in Figs. 8 and 9 clearly show the manner in which the strands entering such terminal are incorporated along 120 with the outer portion of the sleeve and the metal deposited in the mold to form a solid, homogeneous head, presenting all the characteristics of a forged head such as at present 125 employed. It will be understood that if desired such head, especially when of the form resulting from use of a mold such as illustrated in Figs. 3 and 4, may be machined or turned down to present a smooth surface. 130

It will also be noted that the inner portion of the copper sleeve, which is not melted down or welded to the terminal strands, forms a protection for such strands as they 5 emerge, preventing the tendency they otherwise have to break off short, i. e. close to the terminal, as a result of the vibration to which they are subjected in use.

Other forms may be employed embodying 10 the features of my invention instead of the one here explained, change being made in the form or construction, provided the elements stated by any of the following claims or the equivalent of such stated elements be 15 employed, whether produced by my preferred method or by others embodying steps equivalent to those stated in the following claims.

I therefore particularly point out and 20 distinctly claim as my invention:—

1. The method of making a rail-bond of the character described as a separate article of manufacture, which consists in inserting the end of a stranded conductor in a mold- 25 recess of desired shape and size, and then fusing down such inserted end and filling up such recess by means of a metal arc-pencil.

2. The method of making a rail-bond of 30 the character described as a separate article of manufacture, which consists in enclosing the end of a stranded conductor in a sleeve, inserting such end in a mold-recess of desired shape and size, the inner portion of 35 such sleeve being left without such recess, and then fusing down such inserted end along with the outer portion of such sleeve and filling up such recess by means of a metal arc-pencil.

40 3. The method of making a rail-bond of the character described as a separate article of manufacture, which consists in preliminarily compressing the end of a stranded conductor to approximately the cross-section 45 of the desired terminal, inserting such end in a mold-recess of desired shape and size, and then fusing down such inserted end and filling up such recess by means of a metal arc-pencil.

50 4. The method of making a rail-bond of the character described as a separate article of manufacture, which consists in enclosing the end of a stranded conductor in a sleeve, preliminarily compressing such end with 55 sleeve thereon to approximately the cross-section of the desired terminal, inserting such end in a mold-recess of desired shape and size, the inner portion of such sleeve being left without such recess, and then fusing down such inserted end along with the outer portion of such sleeve and filling up such recess by means of a metal arc-pencil.

5. The method of making a rail-bond of 60 the character described as a separate article of manufacture, which consists in enclosing

the end of a stranded copper conductor in a sleeve, likewise of copper, preliminarily compressing such end with sleeve thereon to approximately the cross-section of the desired terminal, inserting such end in a mold-recess of desired shape and size, the inner portion of such sleeve being left without such recess, and then fusing down such inserted end along with the outer portion of such sleeve and filling up such recess by 75 means of a copper arc-pencil.

6. The method of making a rail-bond of the character described as a separate article of manufacture, which consists in inserting the end of a stranded conductor in a mold- 80 recess of desired shape and size, placing in such recess adjacent one wall thereof a metal plate of higher fusibility than said conductor, and then fusing down such inserted end and filling up such recess by means of a metal 85 arc-pencil, said plate being incorporated in one face of the resulting terminal.

7. The method of making a rail-bond of the character described as a separate article of manufacture, which consists in inserting 90 the end of a stranded copper conductor in a mold-recess of desired shape and size, placing in such recess adjacent one wall thereof a plate of ferrous metal, and then fusing down such inserted end and filling 95 up such recess by means of a metal arc-pencil, said plate being incorporated in one face of the resulting terminal.

8. As an independent article of manufacture, a rail-bond having a stranded body and 100 a solid terminal formed of metal molded on the end of said body from a metal arc-pencil, and a metal plate of higher fusibility than said body incorporated in one face of said terminal.

9. As an independent article of manufacture, a rail-bond having a stranded copper body and a solid terminal formed of metal 110 molded on the end of said body from an arc-pencil, substantially as described.

10. As an independent article of manufacture, a rail-bond having a stranded copper body and a solid terminal formed of metal molded on the end of said body from an arc-pencil, and a plate of ferrous metal incorporated in one face of said terminal. 115

11. As an independent article of manufacture, a rail-bond having a stranded body, a sleeve surrounding the end of said body, and a solid terminal formed of metal 120 molded on such end so as to interfuse the component strands of said body and the outer portion of said sleeve.

12. As an independent article of manufacture, a rail-bond having a stranded copper body, a sleeve of copper surrounding the end of said body, and a solid terminal formed of copper molded on such end so as to interfuse the component strands of said body and the outer portion of said sleeve. 125

13. As an article of manufacture, a partially formed bond comprising a stranded conductor, a sleeve surrounding the end of the same and projecting therebeyond to form an enclosure, and braze-material retained in such enclosure.

14. As an article of manufacture, a par-

tially formed bond comprising a stranded copper conductor, a copper sleeve surrounding the end of the same and projecting therebeyond to form an enclosure, and braze-material retained in such enclosure.

Signed by me, this 19 day of June, 1919

CHARLES A. CADWELL